

## UNITED STATES PATENT OFFICE.

THOMAS M. DIVEN, SR., OF BALTIMORE, MARYLAND.

## ACID OR SEA-WATER RESISTING ALLOY.

No Drawing.

Application filed March 25, 1927. Serial No. 178,499.

My invention relates to articles exposed to acids or sea water either water itself or the spray from the water. Heretofore, articles made principally of aluminum and exposed to acids or sea water would decompose and it has been difficult to keep such articles clean or bright looking for any extended length of time. Fish bait, engine bases, and other castings on board ships at sea when made of aluminum, soon tarnish, and in the course of a comparatively short time, are practically ruined by action of the sea water on these exposed articles, yet because of its lightness and its appearance, it has long been desirable to use aluminum articles in fishing tackle and on board vessels at sea, and it is the object of my invention to so treat the aluminum as to render it practically non-tarnishable when exposed to salt water or salt water spray. I have discovered that if these articles are cast from an alloy containing about 93.25% of aluminum, 5.25% of tin, .75% of phosphorus, that the articles will resist the decomposing action of the salt water or spray and will last in their presence for long periods of time without tarnishing.

I have found it also advantageous to incorporate .75% of magnesium into the alloy. The alloy without the magnesium is highly efficient to accomplish the foregoing objects, but is somewhat improved by the addition of the magnesium.

In carrying out my invention, I melt the comparatively pure aluminum in a commercial graphite crucible and add the tin and phosphorus to the melted aluminum and when desirable the magnesium is also added. The alloy is allowed to cool in the ordinary way or if it becomes necessary to roll the

metal, the alloy is first poured into ingots of suitable size for rolling and afterward made into the desired articles.

The addition of the tin, phosphorus and magnesium to the aluminum does not lessen the toughness or malleability of the aluminum or injure its appearance when the articles are made from the alloy so formed, but the alloy has produced quite an unexpected result in withstanding the action of the sea water or spray and the articles made therefrom will retain their properties of toughness or brightness and the other usual properties of aluminum, whereas the pure or commercial aluminum exposed to the same conditions would be tarnished and injured in a short period of time.

I can vary the proportions of the ingredients of my article within the ordinary range of use where alloys of this character are involved, but I prefer approximately the above proportions to get the best described results from the use of my article.

## What I claim is:

1. Articles having the appearance of aluminum and great resistance against the action of acid, salt water or salt water spray, said articles being made from an aluminum alloy containing approximately 5.25% tin, .75% of phosphorus and above 93% aluminum.

2. Articles having the appearance of aluminum and great resistance against the action of acids or salt water, said articles being made from an alloy of aluminum comprising approximately 5.25% tin, .75% phosphorus, .75% magnesium, and the rest aluminum.

In testimony whereof I affix my signature.

THOMAS M. DIVEN, Sr.